



is of lesser importance, the tin content may also be higher. An alloy having a higher tin content is about the following:

|      | Per cent |
|------|----------|
| 5 Pb | 2.5      |
| Sb   | 2.3      |
| Sn   | 5        |
| Al   | Balance  |

10 Since tin alloys weld either with antimony or with lead, it is particularly valuable as addition to the ternary aluminum-lead-antimony-alloy, but also the other metals added to this three-part-alloy result in very useful bearing metals.

15 While the additional metals mentioned above influence chiefly the sliding properties, the further possible additions of at least one of the metals

of the group consisting of copper, nickel, cobalt, iron, manganese and zinc in quantities of 0.1-10% and silicon in quantities of 0.1-3% especially effect a strengthening of the bearing metal which

20 and carbon in quantities of 0.1-3% especially effect a strengthening of the bearing metal which consequently is more suitable to resist higher pressures. Especially an addition of manganese has proved very effective, inasmuch as it not only increases the hardness of the alloy, but even improves essentially the sliding properties. An alloy that proved particularly useful for the auto-

alloy that proved particularly useful for the automobile motor is composed as follows: 2.5% Pb, 2.5% Sb, 3% Mn, remainder Al.

30 Further alloys that correspond about to the properties of the above-mentioned alloys are as follows:

The addition of metals of a higher melting point further serve the purpose of making the bearing metals capable of resisting higher temperatures.

40 metals capable of resisting higher temperatures. While it is correct that with most of the additional metals named above the melting point of aluminum is lowered to the eutectic point, the presence of these metals having higher melting points, more especially if lead and tin with their lower melting point are present, result in the direction of a better resistance to higher tempera-

tures. Bearing temperatures of up to 120° C. could be reached without a clinging or sticking to the axle having occurred. Naturally with such high temperatures the higher heat expansion of the aluminum alloys has to be taken into account by the provision of a greater bearing-play. 5

If the new bearing metals are used under favorable conditions, i. e., presence of ample quantities of lubricants, they show but a small wear, even after a comparatively short running-in period. 10

Summing up, it may be said that with the new bearing metals having an aluminum base as compared with the hitherto known bearing metals, the following advantages exist:

1. Easier running-in.
  2. High resistance to wear.
  3. Possibility of using unhardened axles.
  4. High resistance to temperature.

The alloys may be used in accordance with the invention for any casting method, as sand casting, chill casting, pressure die casting and centrifugal casting. With centrifugal casting the temperatures and numbers of revolutions must be adjusted in such a way that the segregations remain at a minimum. The alloys may further be pressed, forged or rolled. In this respect it is surprising that the annealing in the drawing of rods and tubes may be accomplished at about 500° C. in spite of the lead- and antimony-content without a segregation of the alloys occurring thereby.

For the production of an alloy as uniform as possible, first of all antimony is melted together with aluminum whereupon lead is added as such or as a preliminary alloy. 35

The rolling possibility moreover makes it possible to roll up the alloys to a firmer sheet base that may consist of iron or copper alloys or also of hardenable aluminum alloys and to produce from the compound metal sheets thus obtained especially firm bearing shells.

This application is a division of my copending application, Serial No. 180,029, filed December 15, 1937, now Patent No. 2,196,236, patented April 4, 1940.

I claim:

1. A bearing metal alloy containing about 1-10% of lead, 1-10% of antimony, 0.1-3% of silicon and 0.1-10% of manganese, the balance being substantially all aluminum.
  2. A bearing metal alloy containing about 3% of lead, about 3% of antimony, about 0.3% of silicon, and from 1 to 3% of manganese, the balance being substantially all aluminum.

EUGEN VADER'S